

## UNITED STATES PATENT OFFICE

2,321,501

PRINTING VISCOSE PROCESS RAYON WITH  
ACID AND DIRECT COLORSCharles F. Miller, Wilmington, Del., assignor to  
E. I. du Pont de Nemours & Company, Wil-  
mington, Del., a corporation of DelawareNo Drawing. Application October 25, 1940,  
Serial No. 362,789

6 Claims. (Cl. 8—62)

This invention relates to the printing of acid and direct colors on regenerated cellulose rayon, and especially to improvements which produce prints on regenerated cellulose rayon having superior strength and superior fastness to soaping.

It is among the objects of this invention to provide prints on viscose process rayon made with acid and direct colors which have improved and satisfactory strength and fastness to soaping as compared with the prints heretofore produced on such fabrics. Other objects of the invention will be apparent from the following description.

The objects of the invention are attained in general by incorporating certain assistants into the printing pastes which contain acid and direct colors. These assistants may be present in the proportion of about 3 to about 20 parts of assistant to 3 parts of color and the color may comprise about 1% to about 8% of the paste, the remainder of the paste being constituents which make the composition adaptable for printing with etched rollers or blocks. Such remaining constituents are materials such as textile gums, water or any other desired constituent commonly used in textile pastes. The assistants are hydroscopic agents, being alkali-metal salts of a class of compounds consisting of aliphatic sulfuric and sulfonic acids having 3 to 12 carbon atoms, benzyl thioglycolic acid, alkyl thioglycolic acids in which alkyl has 1 to 12 carbons, aryl sulfonic acids of the benzene and naphthalene series which may be nuclearly substituted once to four times by alkyl having 1 to 8 carbons, halogen, hydroxy or nitro, and mono-esters of the group consisting of the naphthalene dicarboxylic acids and dicarboxylic acids containing not more than 8 carbons of the group consisting of phthalic, aliphatic dicarboxylic acids of the paraffin series and the halogen and hydroxy derivatives of such aliphatic acids and in which the ester groups of said mono-esters are radicals of monohydric alcohols containing not more than 8 carbons of the group consisting of benzyl, allyl, carbocyclic and aliphatic alcohols.

The invention will be more fully set forth in the following more detailed description which includes examples that are given as illustrative embodiments of the invention and not as limitations

thereof. Parts are expressed in parts by weight unless otherwise noted.

## Example I

5 A viscose process rayon fabric was printed with a paste consisting of

|                                  | Parts by weight |
|----------------------------------|-----------------|
| Direct color dyestuff—C. I. #814 | 3.0             |
| Sodium para toluene sulfonate    | 10.0            |
| 10 Water                         | 17.0            |
| Textile gum                      | 70.0            |
|                                  | <hr/> 100.0     |

15 The print was dried, steamed 45 minutes, soaped lightly (3-5 minutes at 110°-120° F.), rinsed and dried. The print was a bright yellow shade. The print was noticeably stronger and faster to soaping than a print made on the same fabric with a similar printing paste which did not contain sodium para toluene sulfonate.

## Example II

A viscose process rayon fabric was printed with a paste consisting of

|                                | Parts by weight |
|--------------------------------|-----------------|
| Acid color dyestuff—C. I. #430 | 3.0             |
| Sodium N-butyl sulfate         | 10.0            |
| Water                          | 17.0            |
| Textile gum                    | 70.0            |
|                                | <hr/> 100.0     |

25 The printed rayon was dried, aged 45 minutes by steaming, soaped lightly, rinsed and dried. The printing was an even brilliant red design. It was stronger and faster to soaping than one made on the same kind of fabric with a similar printing paste which did not contain sodium N-butyl sulfate.

## Example III

30 Viscose process rayon fabric was printed with a paste consisting of

|                                  | Parts by weight |
|----------------------------------|-----------------|
| Direct color dyestuff—C. I. #319 | 3.0             |
| Sodium benzyl thioglycolate      | 7.5             |
| Water                            | 19.5            |
| Textile gum                      | 70.0            |
|                                  | <hr/> 100.0     |

35 The print was steamed, soaped and finished as

described in Example I. The print was a brilliant violet design which was stronger and faster to soaping than a print made in the same way on the same kind of fabric with a similar paste except that the latter paste did not contain sodium benzyl thioglycolate.

Any acid color or any direct color can be used as the color constituent in the new pastes with similar improvement in result. As illustrations of such dyestuffs the following are mentioned: direct color dyestuffs Color Index numbers 813, 561, 581, 812, 620, 816 and acid color dyestuffs Color Index numbers 307, 289, 666, 670, 1088 and 1080. As representative of other soluble salts of the described class of assistants which can be used with any of the direct or acid colors to produce similar improved results are mentioned the sodium and potassium salts of N-octyl sulfate, N-propyl sulfate, isopropyl sulfate, para phenol sulfonate, tetralin sulfonate, alpha naphthalene sulfonate, methyl adipate, benzyl succinate, isobutyl sulfate, N-butyl sulfonate, p-nitro benzene sulfonate, o-chlortoluene sulfonate, N-propyl thioglycolate, lauryl sulfate, methyl thioglycolate, n-hexyl thioglycolate, octyl thioglycolate, lauryl thioglycolate, and the methyl, ethyl, propyl, isopropyl, butyl, isobutyl, amyl, n-hexyl, ethyl butyl, ethyl hexyl, benzyl, chlor benzyl, phenyl ethyl, cyclohexanyl, octyl and allyl mono-esters of phthalic, naphthalene-o-dicarboxylic, naphthalic, oxalic, malonic, adipic, methyl adipic, succinic, methyl succinic, dimethyl succinic, chlor malonic, tartaric and suberic acids.

The preferred assistants are the alkali-metal salts of the indicated alkyl sulfuric acids, the alkyl- and benzyl-thioglycollic acids and mono-esters of the dicarboxylic acids.

In the foregoing examples the ratio of dyestuff to assistant in the paste is 3 to 10 by weight, but other proportions can be used. This proportion can be varied with 3 parts of color from about 3 parts to about 20 parts of assistant. The proportion of water textile gum and other constituents can be varied within any desired limits which will enable the paste to be used for the purpose of printing fabrics by the use of etched rollers and like appliances. The proportion of textile gum and water can be varied within any limits which will give the printing paste a suitable viscosity for printing. Any textile gum suitable for this purpose can be used, such as gum tragacanth, starch, locust bean gum, gum karaya, gum arabic, dextrin, agar, vegetable colloid and various mixtures of such materials. More or less of the thickening agent will be required in order that the printing paste will have a suitable viscosity to operate satisfactorily on the etched roller or other printing device. The proportion can be widely varied and determined by experiment according to various circumstances, such as the characteristics of the printing member and the material upon which the prints are to be disposed.

From the foregoing disclosure it will be recog-

nized that the invention is susceptible of modification without departing from the spirit and scope thereof and it is to be understood that the invention is not restricted to the specific illustrations thereof herein set forth.

I claim:

1. A printing paste which comprises a dyestuff of a group consisting of direct and acid colors, a hydrous thickening agent in sufficient amount to enable the paste to be printed on a viscose rayon fabric and an assistant of a group consisting of an alkali-metal salt of a group consisting of the benzyl and alkyl thioglycollic acids in which alkyl has 1 to 12 carbons, said dyestuff being present in the proportion of about 1.0% to about 8.0% of the paste and the ratio of dyestuff to assistant being about 3 parts of dyestuff with about 3 parts to about 20 parts of said assistant.
2. A printing paste which comprises a dyestuff of a group consisting of direct and acid colors, a hydrous thickening agent in sufficient amount to enable the paste to be printed on a viscose rayon fabric and an alkali-metal benzyl thioglycolate, the dyestuff and said assistant being present in the proportion of about 3 parts by weight of dyestuff to about 10 parts by weight of said assistant.
3. The process which comprises printing on a viscose rayon fabric with a printing paste which comprises a dyestuff of a group consisting of direct and acid colors, a hydrous thickening agent in sufficient amount to enable the paste to be printed on a viscose rayon fabric, and an alkali-metal benzyl thioglycolate; drying the print and then steaming until the print is developed.
4. A printing paste which comprises a dyestuff of a group consisting of direct and acid colors, a hydrous thickening agent in sufficient amount to enable the paste to be printed on a viscose rayon fabric and sodium benzyl thioglycolate, the dyestuff and said assistant being present in the proportion of about 3 parts by weight of dyestuff to about 10 parts by weight of said assistant.
5. The process which comprises printing on a viscose rayon fabric with a printing paste which comprises a dyestuff of a group consisting of direct and acid colors, a hydrous thickening agent in sufficient amount to enable the paste to be printed on a viscose rayon fabric and an assistant of a group consisting of an alkali-metal salt of a group consisting of benzyl and alkyl thioglycollic acids in which alkyl has 1 to 12 carbons, drying the print and then steaming until the print is developed.
6. The process which comprises printing on a viscose rayon fabric with a printing paste which comprises a dyestuff of a group consisting of direct and acid colors, a hydrous thickening agent in sufficient amount to enable the paste to be printed on a viscose rayon fabric, and sodium benzyl thioglycolate; drying the print and then steaming until the print is developed.

CHARLES F. MILLER.